

# United States Patent [19]

Fanelli et al.

[11] Patent Number: 4,787,989

[45] Date of Patent: Nov. 29, 1988

[54] ANIONIC SOIL RELEASE COMPOSITIONS

[75] Inventors: Joseph J. Fanelli, Alpharetta; Randy L. Rayborn, Winder; Donald Jenkins, Duluth; Anthony J. O'Lenick, Jr., Lilburn, all of Ga.

[73] Assignee: GAF Corporation, Wayne, N.J.

[21] Appl. No.: 143,581

[22] Filed: Jan. 13, 1988

[51] Int. Cl.<sup>4</sup> ..... D06M 00/00; C11D 3/37; C11D 1/00

[52] U.S. Cl. ..... 252/8.6; 252/807; 252/8.9; 252/174.19; 252/174.25; 252/DIG. 15; 252/174.23; 528/272; 528/274; 528/296; 528/339

[58] Field of Search ..... 252/8.6, 8.7, 8.9, 174.19, 252/174.25, DIG. 15; 528/272, 274, 296, 339

[56] References Cited

U.S. PATENT DOCUMENTS

3,959,230 5/1976 Hays ..... 252/8.9

|           |         |                       |          |
|-----------|---------|-----------------------|----------|
| 4,125,370 | 11/1978 | Nizol .....           | 252/8.9  |
| 4,225,646 | 9/1980  | Cushion, Jr. .....    | 252/8.9  |
| 4,233,436 | 11/1980 | Robinson .....        | 528/366  |
| 4,257,928 | 3/1981  | Vachon et al. .....   | 524/386  |
| 4,268,645 | 5/1981  | Lark .....            | 525/437  |
| 4,611,021 | 9/1986  | Zamek .....           | 524/317  |
| 4,711,730 | 12/1987 | Goselink et al. ..... | 252/8.75 |

Primary Examiner—Robert Wax

Assistant Examiner—Ronald A. Krasnow

Attorney, Agent, or Firm—Marilyn J. Maue; Joshua J. Ward

[57]

## ABSTRACT

The present invention relates to a class of compounds which have superior soil release properties over heretofore known soil release polymers. The compounds are prepared by the reaction of an aromatic hydroxy containing polyester soil release agent with trimellitic anhydride under acid catalysis to produce an aromatic terminal capped carboxyloxy soil release polymer.

12 Claims, No Drawings

## ANIONIC SOIL RELEASE COMPOSITIONS

## BACKGROUND OF THE INVENTION

The present application relates to anionic block polyesters useful as soil release and antistatic agents. In addition to cleaning performance, laundry detergent compositions should have other benefits. One is the ability to impart soil release properties to fabrics woven from polyester and other fibers. These fabrics are predominantly co-polymers of ethylene glycol and terephthalic acid, and are sold under a number of trade names, e.g., Dacron, Fortrel, Kodel and Blue C Polyester. The hydrophobic character of polyester fabrics makes their laundering difficult, particularly with oily soil and oily stains. The oily soil or stain preferentially "wets" the fabric. As a result, the oily soil or stain is difficult to remove in an aqueous laundering process.

Products which have been used for their soil release and antistatic agents properties can be divided into several classes based upon the chemistry of the products.

Polyesters containing random ethylene terephthalate/polyethylene glycol (PEG) terephthalate units

High molecular weight (e.g., 40,000 to 50,000 M.W.) polyesters containing random ethylene terephthalate/polyethylene glycol (PEG) terephthalate units have been used as soil release compounds in laundry detergent compositions. U.S. Pat. No. 3,962,152 to Nicol et al, issued June 8, 1976. During the laundering operation, these soil release polyesters adsorb onto the surface of fabrics immersed in the wash solution. The adsorbed polyester then forms a hydrophilic film which remains on the fabric after it is removed from the wash solution and dried. This film can be renewed by subsequent washing of the fabric with a detergent composition containing the soil release polyesters.

These ethylene terephthalate/PEG terephthalate polyesters are not water-soluble. It is believed that they form a suspension in the wash solution which does not adsorb efficiently onto the fabrics. As a result, the level of soil release polyester in the detergent composition has to be increased if benefits are to be obtained after several wash cycles. Because of this poor water-solubility, these polyesters are formulated as suspensions in laundry detergent compositions, rather than as isotropic liquids. In certain detergent formulations, these polyesters can also diminish clay soil cleaning performance.

Polyester antistatic agents formed from dimethyl terephthalate, ethylene glycol and methoxy PEGs

U.S. Pat. No. 3,416,952 to McIntyre et al., issued Dec. 17, 1968, discloses the treatment of shaped polyester articles with a water-insoluble crystallizable polymeric compound which can contain a water soluble polymeric group such as a polyoxyalkylene group having an average molecular weight of from 300-6000. Preferred polyoxyalkylene groups are the PEGs having an average molecular weight of from 1000-4000. Treatment of the shaped articles is carried out by applying an aqueous dispersion of the crystallizable polymeric compound in the presence of an anti-oxidant, followed by heating to a temperature above 90 degrees C. to obtain a durable coating of the compound on the shaped article. One such crystallizable polymeric compound is formed by the reaction of dimethyl terephthalate, ethyl-

ene glycol and an O-methyl poly-(oxyethylene) glycol of average molecular weight 350. A 20% solution of this polyester in benzyl alcohol was used to impart antistatic properties to a polyester fabric. The patent also discloses a 20% aqueous solution of a similar polyester used to impart antistatic properties to a polyester fabric.

Polyester antistatic and soil release agents formed from dimethyl terephthalate, sodium dimethyl-5-sulfoisophthalate, ethylene glycol and polyethylene glycol (PEG)

U.S. Pat. No. 4,427,557 to Stockburger, Jan. 24, 1984, discloses low molecular weight copolymers (M.W. 2,000 to 10,000) which can be used in aqueous dispersions to impart soil release properties to polyester fibers. The copolymers are formed by the reaction of ethylene glycol, a PEG having an average molecular weight of 200 to 1000, an aromatic dicarboxylic acid (e.g., dimethyl terephthalate), and a sulfonated aromatic dicarboxylic acid (e.g., dimethyl 5-sulfoisophthalate). The PEG can be replaced in part with monoalkylethers of PEG such as the methyl, ethyl and butyl ethers. A dispersion or solution of the copolyester is applied to the textile material and then heat set at elevated temperatures (90 degrees to 150 degrees C.) to impart durable soil release properties.

Monomeric polyesters of PEG and terephthalic acid useful as soil release agents

U.S. Pat. No. 4,349,688 to Sandler, issued Sept. 14, 1982, discloses polyoxyalkylene phthalate ester soil release agents.



Durable soil resistance and water wicking properties are imparted by wetting the fabric with a composition containing the polyoxyalkylene ester, drying the wetted fabric, and then curing the dried fabric at a temperature of from 190-200 degrees C. for about 45-90 seconds.

Ethylene terephthalate/PEG terephthalate soil release polyesters for fabric treating solutions

U.S. Pat. No. 3,959,230 to Hays, issued May 25, 1976, discloses polyester soil release agents containing random ethylene terephthalate/PEG terephthalate units in a mole ratio of from about 25:75 to about 35:65. These soil release polyesters have a molecular weight of from about 25,000 to about 55,000, (preferably from about 40,000 to about 55,000) and are used in dilute, aqueous solutions, preferably with an emulsifying agent present. Fabrics are immersed in this solution so that the soil release polyester adsorbs onto the fabric surface. The polyester forms a hydrophilic film which remains on the fibers after the fabric is removed from the solution and dried. See also U.S. Pat. No. 3,893,929 to Basadur, issued July 8, 1975 (compositions for imparting soil release finish containing a polyester having an average molecular weight of 3000-5000 formed from terephthalic acid, PEG and ethylene glycol); U.S. Pat. No.

3,712,873 to Zenk, issued Jan. 23, 1973 (textile treating composition comprising fatty alcohol polyethoxylates; quaternary ammonium compounds; a polyester having average molecular weight of 3000-5000 formed from terephthalic acid, PEG and ethylene glycol; and starch).

Ethylene terephthalate/PEG terephthalate soil release agents used in detergent compositions

U.S. Pat. No. 3,962,152 to Nicol et al., issued June 8, 1976, discloses detergent compositions containing detergent surfactants and the ethylene terephthalate/PEG terephthalate soil release polyesters disclosed in U.S. Pat. No. 3,959,230 issued to Hays. Additionally U.S. Pat. No. 4,116,885 to Derstadt et al., issued Sept. 26, 1978 (detergent compositions containing certain compatible anionic detergent surfactants and ethylene terephthalic/PEG terephthalate soil release polyesters); U.S. Pat. No. 4,132,680 to Nicol, issued Jan. 2, 1979 (detergent compositions containing detergent surfactants; a composition which disassociates to yield quaternary ammonium cations; and an ethylene terephthalate/PEG terephthalate soil release polyester) are of interest.

Soil release and antistatic polyurethanes useful in detergent compositions which contain polyester blocks having sulfoisophthalate units

U.S. Pat. No. 4,201,824 to Violand et al., issued May 6, 1980, discloses hydrophilic polyurethanes having soil release and antistatic properties useful in detergent compositions. These polyurethanes are formed from the reaction product of a base polyester with an isocyanate prepolymer (reaction product of diisocyanate and macrodioil). Further, a disclosure of base polyester formed from dimethyl terephthalate, dimethyl sulfoisophthalate, ethylene glycol and PEG (molecular weight 300) which is reacted with a prepolymer formed from a PEG (molecular weight 1,500) and toluene diisocyanate is made.

The previously mentioned patents, included by reference, describe a number of ways that one can make polymeric materials which are substantive to fiber. This substantivity renders the fiber soil resistant.

One shortcoming of these polyester type polymers used as soil release materials is that the benefits of softening and hand modification desired by the consumer are not realized. Softeners are typically formulated into detergents or added in a post step as a rinse cycle softener.

Additionally, U.S. Pat. No. 4,134,839 to Marshall discloses the use of an alkanolamide reacted with a polycarboxybenzene ester to give a soil release polymer.

U.S. Pat. No. 4,375,540 to Joyner discloses copolyester derivatives from aromatic dibasic acid and aliphatic dibasic acids of glycol.

U.S. Pat. No. 4,310,426 to Smitz discloses a yellowing resistant soil release agent.

U.S. Pat. No. 4,094,796 to Schwarz discloses a novel polyoxyalkylene polymeric.

## THE INVENTION

It is the objective of this invention to provide both soil release and antistatic properties. More specifically, the present invention is directed to certain polyoxyalkylene ester carboxylates and the preparation and application of said polyoxyalkylene ester carboxylates. The

presence of a terminal carboxyloxy group improves the soil release properties over more conventional soil release agents. The terminal position and the carboxyloxy nature are very important to the functionality of the molecule. We have determined that the choice of catalyst used in the reaction can have a profound effect upon where the hydroxyl group reacts. This in turn has a dramatic effect upon hydrolytic stability and performance.

Trimellitic anhydride has the following structure;



We have discovered that when an acidic catalyst like paratoluene sulfonic acid is used, the anhydride functionality is maintained and reaction occurs at the carboxyl group in the 5 position of the aromatic ring. The fact that water is distilled off under reaction conditions confirms that the anhydride did not react. If the anhydride had in fact opened there would be no distillate. Additionally, the presence of the anhydride is confirmed by Infra Red analysis 1780 cm<sup>-1</sup> and wet analysis.

Percentages and ratios used herein are by weight, unless otherwise noted. References cited herein are incorporated by reference.

## DETAILED DESCRIPTION OF THE INVENTION

The compounds of the invention conform to the following generic structure;



R'' is



Q is H or SO3Na; X is H or CH<sub>3</sub>  
a is an integer from 1-5; b is an integer from 1-200  
preferably from 1-20  
c is an integer from 1-50 preferably from 1-10; M is  
Na, H, K, Li, NH4

The compounds of this invention can be formulated into products that are applied directly in aqueous solution by themselves or formulated with anionics or non-ionics and builders to prepare finished conditioner/detergent systems. The following data demonstrates that 5

Q is a mixture of hydrogen and SO<sub>3</sub>Na  
 X is H and/or CH<sub>3</sub>  
 a is an integer from 1-5  
 b is an integer from 1-200  
 c is an integer from 1-50



the compounds of the present invention provide desirable properties when compared to commercially available products. Rating System 1 is worst 5 is best. Soil Release was tested on polyester fabrics using AATCC Method 130. These tests are used to evaluate the ability of a compound to release oily soils during home laundering. Values 2 and below are considered non performing. 15

15

20

25

30

35

40

45

50

55

60

65

70

75

80

85

90

95

100

105

110

115

120

125

130

135

140

145

150

155

160

165

170

175

180

185

190

195

200

205

210

215

220

225

230

235

240

245

250

255

260

265

270

275

280

285

290

295

300

305

310

315

320

325

330

335

340

345

350

355

360

365

370

375

380

385

390

395

400

405

410

415

420

425

430

435

440

445

450

455

460

465

470

475

480

485

490

495

500

505

510

515

520

525

530

535

540

545

550

555

560

565

570

575

580

585

590

595

600

605

610

615

620

625

630

635

640

645

650

655

660

665

670

675

680

685

690

695

700

705

710

715

720

725

730

735

740

745

750

755

760

765

770

775

780

785

790

795

800

805

805

810

815

820

825

830

835

840

845

850

855

860

865

870

875

880

885

890

895

900

905

910

915

920

925

930

935

940

945

950

955

960

965

970

975

980

985

990

995

1000

1005

1010

1015

1020

1025

1030

1035

1040

1045

1050

1055

1060

1065

1070

1075

1080

1085

1090

1095

1100

1105

1110

1115

1120

1125

1130

1135

1140

1145

1150

1155

1160

1165

1170

1175

1180

1185

1190

1195

1200

1205

1210

1215

1220

1225

1230

1235

1240

1245

1250

1255

1260

1265

1270

1275

1280

1285

1290

1295

1300

1305

1310

1315

1320

1325

1330

1335

1340

1345

1350

1355

1360

1365

1370

1375

1380

1385

1390

1395

1400

1405

1410

1415

1420

1425

1430

1435

1440

1445

1450

1455

1460

1465

1470

1475

1480

1485

1490

1495

1500

1505

1510

1515

1520

1525

1530

1535

1540

1545

1550

1555

1560

1565

1570

1575

1580

1585

1590

1595

1600

1605

Additionally products containing both EO and PO can be made by substituting an ethylene oxide/propylene oxide polymer of the same molecular weight for the polyoxyethylene material above.

C

30.0 parts of dimethyl terephthalate, 10.0 parts of ethylene glycol along with 170 parts of polyethylene glycol of nominal molecular weight 4000 and antimony trioxide (0.0022 parts) were charged to a 4-necked flask with a scaled bottom runoff tube and fitted with a stirrer, internal thermometer, nitrogen inlet and a condenser set for distillation. The flask was heated in an electric mantle through which the bottom runoff tube protruded. The temperature of the contents of the flask was raised to 260 degrees plus/minus 5 degrees C. over half an hour and held at 260 degrees C. plus/minus C. for three hours.

Additionally products containing both EO and PO can be made by substituting an ethylene oxide/propylene oxide polymer of the same molecular weight for the polyoxyethylene material above.

D

Spinning grade poly-(ethylene terephthalate) (134.4 parts) a block polymer (2:1 ethylene oxide to propylene oxide having a molecular weight of 1540 MWU) (308 parts) and antimony trioxide (0.0022 part) were charged to a 4-necked flask with a scaled bottom runoff tube and fitted with a stirrer, internal thermometer, nitrogen inlet and a condenser set for distillation. The flask was heated in an electric mantle through which the bottom runoff tube protruded. The temperature of the contents of the flask was raised to 260 degrees plus/minus 5 degrees C. over half an hour and held at 260 degrees C. plus/minus 5 C.

### EXAMPLES

#### General Procedure

Into a suitable reaction flask, equipped with a thermometer, nitrogen sparge and agitator is added the specified amount of raw material polymer (selected from examples 1-3). The raw material polymer is heated to 100 degrees C., under a nitrogen sparge. The specified amount of para toluene sulfonic acid is then added. Next, the specified amount of trimellitic anhydride is then added over a fifteen minute period under good agitation. Heat to 200 C. and hold for 6 to 10 hours.

| Example Number | Raw Material Method | Polymer Weight in Grams | p-Toluene Sulfonic Acid Weight in Grams | Tri mellitic Anhydride Weight in Grams |
|----------------|---------------------|-------------------------|-----------------------------------------|----------------------------------------|
| 1              | B                   | 875.0                   | 2.0                                     | 123.0                                  |
| 2              | C                   | 920.0                   | 2.0                                     | 78.0                                   |
| 3              | A                   | 953.0                   | 1.5                                     | 145.0                                  |
| 4              | D                   | 850.0                   | 2.0                                     | 148.0                                  |

#### EXAMPLE #5

A aqueous solution containing 0.1 to 1.0% active of one of the novel compounds selected from the above examples (1 to 4) are applied to a cotton polyester blend or fiber by exhaustion or using conventional dip and nip technology. The novel compound acts as a lubricant for

the processing of the fiber and a superior soil release agent.

#### EXAMPLE #6

5 A solution of 0.25-1.50% active of one of the compounds above is applied to a polyester blend by exhaustion or using conventional dip and nip technology. The material acts as a lubricant for the processing of the fiber and a non-yellowing softener.

What is claimed:

1. A detergent composition comprising a surfactant and an effective soil releasing amount of a compound having the formula



30 wherein

R is



40 Q is selected from the group consisting of H and SO<sub>3</sub>Na

45 X is H or CH<sub>3</sub>

a is an integer from 1-5

b is an integer from 1-200

c is an integer from 1-50

45 M is selected from the group consisting of Na, H, K, Li and NH<sub>4</sub>.

2. The composition of claim 1 wherein Q is H.

3. The composition of claim 1 wherein Q is SO<sub>3</sub>Na.

4. The composition of claim 1 wherein X is CH<sub>3</sub>.

5. The composition of claim 1 wherein X is H.

6. The composition of claim 1 wherein R is



7. The composition of claim 1 wherein R is



8. The composition of claim 1 wherein R is a blend of



- 10 9. The composition of claim 1 wherein Q is a blend of hydrogen and  $\text{SO}_3\text{Na}$ .  
 10. The composition of claim 1 wherein b is an integer from 1-20 and c is an integer from 1-10.  
 11. A process for contacting a fibrous or keratinous  
 15 with an effective soil releasing amount of the composition of claim 1.

12. The process of claim 11 wherein the substrate is polyester.

\* \* \* \* \*

20

25

30

35

40

45

50

55

60

65